

Oct. 31, 1933.

O. LAUBI

1,933,019

METHOD OF MANUFACTURING ARTIFICIAL TEXTILES

Filed Nov. 30, 1931

Fig. 1.



Fig. 2.



Fig. 3.

Invantor  
Otto Laubi

By A. F. Wendell  
Atty

## UNITED STATES PATENT OFFICE

1,933,019

METHOD OF MANUFACTURING ARTIFICIAL  
TEXTILES

Otto Laubi, Basel, Switzerland, assignor to the  
firm of Lonza Elektrizitätswerke und Chem-  
ische Fabriken Aktiengesellschaft, Basel,  
Switzerland

Application November 30, 1931, Serial No.  
578,196, and in Switzerland December 9, 1930

15 Claims. (Cl. 18—54)

The object of the present invention is a process for making artificial textiles, as for example hollow threads, tube- or hose-like bodies, artificial straw, flat strips and the like.

5 It has already been proposed (see for example the French Patent No. 430,939) to make tubular straw-like material and the like by spinning solutions of nitro-cellulose, cellulose acetate, copper oxide ammonium cellulose, cellulose xanthate 10 and the like through spinnerets with annular apertures. Hereby, by means of an electrically heated core, arranged concentrically in the annular opening, an immediate coagulation of the inner wall of the tubular body is effected, to prevent its sticking together. The great difficulties 15 met with in the technical employment of this process have prevented its achieving a practical value.

It has also been proposed to make hollow 20 threads of cellulose acetate by spinning a solution of acetate of about 10% strength in acetic acid into an aqueous precipitating bath, the thread traversing in its precipitation a path of about two meters. According to this process, 25 however, only more or less flat hollow threads of opaque appearance can be made (see for example British Patent No. 239,622).

Further it is known to make straw substitute, 30 and artificial tubes or hoses from viscose or the like by acting with precipitating baths upon the outer wall, or simultaneously upon the outer and inner walls of a tubular body spun through an annular aperture. It has further been proposed to spin solutions of cellulose or cellulose esters 35 through slit shaped openings into precipitating baths and to twist one or more of the strips so obtained to produce a body which has also been termed artificial straw. In this way, however, only a sort of helical tubes which more or less 40 easily become untwisted can be obtained, because the edges of the single strips so united are not, or only but slightly, joined together.

Finally it is known to produce tubular bodies 45 of such kind with a thread-like core or inlay. The process described below forming the subject of the present invention distinguishes from the above wet spinning methods by the feature that the forming of the products is effected by the dry method, and further by the use, not as 50 hitherto of a more or less easy flowing solution, but of a mass of such concentration that will, after its extrusion from the nozzle, harden more or less rapidly also on the inside of the hollow thread or tube, and finally by the feature that 55 the bodies produced by the present process are

of ring-like closed cross-section and accordingly no untwisting of the bodies or separating into single strips is possible.

According to the invention artificial textiles, as for example hollow threads, tube- or hose-like 60 bodies, artificial straw, flat strips and the like are prepared from cellulose acetate or other cellulose esters or cellulose ethers or mixtures thereof by the raw material being used in the form of highly concentrated dough-like solutions or 65 masses flowing only with difficulty or not at all at ordinary temperatures, which contain at least about 30% of cellulose derivative and if desired softening agents. These solutions or masses are pressed, according to the invention, under high 70 pressure, for example up to say 300 atmospheres or more, and advantageously under heat through a nozzle or nozzles with annular discharge orifices, whilst at the same time through one or more 75 bores arranged within the nozzle air or another gas, together with one or more thread-like inlays, for example textile threads, metal wires or the like are introduced into the interior of the extruded body. Thus the air or gas stream prevents in all cases a collapse of the spun hollow 80 body at the exit from the nozzle, whilst ensuring exact formation of the inner wall of the tube-like body.

The thread-like inlay or inlays are enclosed in this operation in a joint-less covering of cellulose 85 ester or ether which can be of varying thickness and form, for example circular, oval, polygonal and so forth and may firmly, slightly or not at all adhere to the inlay or inlays according to the materials and working conditions chosen. In all 90 cases, the introduced air or other gas stream involves the formation of a hollow space remaining clear within the body.

The process according to the present invention 95 can be carried out by the use of particular nozzles of which Figures 1, 2 and 3 of the accompanying drawing show some types in vertical section. Figure 1 shows a nozzle with an annular discharge orifice *a* for the fluid cellulose mass and a central bore *b* for the passage of a thread-like inlay *c* and 100 air or gas introduced at *e* into a vessel *f* communicating with said bore *b*.

A similar nozzle is represented by Figure 2, wherein the central bore *b* placed within the annular nozzle discharge orifice *a* is sufficiently enlarged to allow the simultaneous passage of three thread-like inlays *c* together with an air stream. 105

In Figure 3 a nozzle is shown which comprises four bores *b* for the passage of four thread-like 110

inlays *c*, whilst a separate bore *g* is provided for the passage of a central air stream.

It has been found that a particularly intimate connection between the thread-like inlay and the jointless covering can be obtained by impregnating or covering the textile thread or threads or wire or wires with a suitable plastic mass before passing them through the nozzle. This can be effected for example by a preliminary treatment 10 of the threads or wires with a cellulose acetate solution containing one or more softening agents and subsequent more or less complete drying. To the same end the threads or wires can be previously treated with advantageously small quantities 15 of substances acting as solvents or swelling agents on the covering material, for example with tri-acetine if the covering is to be of cellulose acetate.

With the use for example of cellulose acetate 20 threads as the inlay and a covering of the same material, the covering adheres very firmly to the inlay without preliminary treatment of the latter being necessary.

The solutions or masses to be worked with under 25 the invention can be prepared with suitable low or high boiling solvents or solvent mixtures as for example acetone and/or triacetine, or with mixtures of solvents and non-solvents. Mixtures of liquids can also be used which alone do not dissolve 30 the cellulose derivatives, but when mixed do so.

The content of cellulose derivatives or of these 35 together with the softening agents in the masses to be used under the invention, should, as above mentioned, be so high that the masses at ordinary temperature will flow only with difficulty or not at all and have a consistency say of a more or less stiff dough.

With cellulose acetate solutions free of softening 40 agents the uppermost limit may be about 70% and more and the lowest limit about 30% of acetate. For example solutions containing 50% of cellulose acetate and 50% of acetone or in place of the latter 50% of a mixture of methylene 45 chloride and alcohol (3:1) are very suitable.

The addition of solid or liquid softening agents or of mixtures of solid and liquid softening agents 50 is of advantage. By means of these, the acetate content of the solutions or masses can be reduced. The acetate content should however not fall below about 30%.

Solutions or masses which contain no softening 55 agents yield hard, but slightly flexible final products of considerable tearing strength. With the addition of softening agents, they yield more or less soft, elastic and flexible final products.

By the addition of finely divided filling materials, as for instance barium sulphate, gold bronze 60 or other fine metal powders, pigments, dissolved or dispersed dyestuffs, solutions or emulsions of oily substances or the like, or by additions such as are used or have been proposed for example in the manufacture of artificial silk, there can be 65 given to the end products of the present process determined properties or a particular appearance, for instance a matt appearance. By the addition of substances which lead during the forming 70 process to a weak gas development, for example by impregnation of the masses with air or carbon dioxide, end products of the nature of the so-called air-silk containing fine bubbles can be obtained.

75 The quality of the final products may be im-

proved by filtering the solutions or masses before they are worked up.

The forming of the solutions or masses into hollow threads, tubes or hoses or the like is effected, as mentioned above, by pressing them through annular nozzle orifices, whilst a gas, for example air, in cold, warm or hot condition, is simultaneously discharged under the necessary pressure into the interior of the extruded body to prevent collapse of the tube or the like.

According to the present process it is possible to make artificial straw with inlay of most varying diameters, for example from 0.2 to 10 mm. and more.

It may be noted that according to the quantity 90 of air or gas pressed in during the formation of the body, straws or the like will be obtained of circular or more or less flat cross-section. If little air is supplied, flat bands can be produced which are also a usable product, for example in 95 the textile industry.

In the manufacture according to the invention of artificial straw or the like with reinforcing inlays, one or more cotton threads, hemp threads, paper threads or the like, twisted together or not, or cords or artificial threads, for example of cellulose acetate, can be used. Further, for example cotton covered wires can have cellulose derivative masses expressed round them according to the invention. To obtain 105 special effects the inlay threads can be coloured all the same or differently one from another while using an uncoloured covering mass.

In order to obtain flat pressed, easily flexible 110 artificial straw or the like, the fully or not yet entirely dried, if necessary resoftened, bodies can be led between or operated upon by rollers which can be smooth or longitudinally or circumferentially corrugated. Further, characters or ornaments can in this way be pressed into the 115 bodies or printed thereon with colours.

The products obtainable by the process according to the present invention, for example 120 hollow threads, bands and so forth, in particular the manifold kinds of artificial straw obtainable thereby with inlays of textile threads or wires or the like will chiefly find employment for plaited work, for example for hat and basket work making; but they can also be used for making cords or ropes and in so far as they can be spooled they 125 can also be used for weaving.

What I claim is:—

1. A process for making artificial textiles such as hollow threads, tube- or hose-like bodies, artificial straw, flat strips and the like from esters 130 and/or ethers of cellulose, according to the dry method, comprising forcing highly concentrated, dough-like solutions or masses flowing only with difficulty or not at all at ordinary temperature, and containing at least about 30% of cellulose 135 derivative, through nozzles with annular orifices under high pressure, while simultaneously jointly introducing at least one thread-like inlay and a gas stream into the body in formation.

2. A process for making artificial textiles such 140 as hollow threads, tube- or hose-like bodies, artificial straw, flat strips and the like from esters and/or ethers of cellulose, according to the dry method, comprising forcing highly concentrated dough-like solutions or masses flowing only with difficulty or not at all at ordinary temperature, and containing at least about 30% of cellulose 145 derivative, and at least one solid softening agent, through nozzles with annular orifices under high pressure, while simultaneously jointly introduc- 150

- ing at least one thread-like inlay and a gas stream into the body in formation.
3. A process for making artificial textiles such as hollow threads, tube- or hose-like bodies, artificial straw, flat strips and the like from esters and/or ethers of cellulose, according to the dry method, comprising forcing highly concentrated, dough-like solutions or masses flowing only with difficulty or not at all at ordinary temperature, and containing at least about 30% of cellulose derivative, through nozzles with annular orifices under a pressure up to about 300 atmospheres or more, while simultaneously jointly introducing at least one thread-like inlay and a gas stream into the body in formation.
4. A process for making artificial textiles such as hollow threads, tube- or hose-like bodies, artificial straw, flat strips and the like from esters and/or ethers of cellulose, according to the dry method, comprising forcing highly concentrated, dough-like solutions or masses flowing only with difficulty or not at all at ordinary temperature, and containing at least about 30% of cellulose derivative and at least one liquid softening agent, through nozzles with annular orifices under high pressure, while simultaneously jointly introducing at least one thread-like inlay and a gas stream into the body in formation.
5. A process for making artificial textiles such as hollow threads, tube- or hose-like bodies, artificial straw, flat strips and the like from esters and/or ethers of cellulose, according to the dry method, comprising forcing highly concentrated, dough-like solutions or masses flowing only with difficulty or not at all at ordinary temperature, and containing at least about 30% of cellulose derivative and a mixture of solid and liquid softening agents, through nozzles with annular orifices under high pressure, while simultaneously jointly introducing at least one thread-like inlay and a gas stream into the body in formation.
6. A process for making artificial textiles such as hollow threads, tube- or hose-like bodies, artificial straw, flat strips and the like from esters and/or ethers of cellulose, according to the dry method, comprising forcing highly concentrated, dough-like solutions or masses flowing only with difficulty or not at all at ordinary temperature, and containing at least about 30% of cellulose derivative and filling substances, through nozzles with annular orifices under high pressure, while simultaneously jointly introducing at least one thread-like inlay and a gas stream into the body in formation.
7. A process for making artificial textiles such as hollow threads, tube- or hose-like bodies, artificial straw, flat strips and the like from esters and/or ethers of cellulose, according to the dry method, comprising forcing highly concentrated, dough-like solutions or masses flowing only with difficulty or not at all at ordinary temperature, and containing at least about 30% of cellulose derivative, through nozzles with annular orifices under high pressure, while simultaneously jointly introducing at least one thread-like inlay and an air stream into the body in formation.
8. A process for making artificial textiles such as hollow threads, tube- or hose-like bodies, artificial straw, flat strips and the like from esters and/or ethers of cellulose, according to the dry method, comprising forcing highly concentrated, dough-like solutions or masses flowing only with difficulty or not at all at ordinary temperature, and containing at least about 30% of cellulose derivative, through nozzles with annular orifices under high pressure, while simultaneously introducing at least one thread-like inlay and a gas stream into the body in formation.
9. A process for making artificial textiles such as hollow threads, tube- or hose-like bodies, artificial straw, flat strips and the like from esters and/or ethers of cellulose, according to the dry method, comprising forcing highly concentrated, dough-like solutions or masses flowing only with difficulty or not at all at ordinary temperature, and containing at least about 30% of cellulose derivative, through nozzles with annular orifices under high pressure, while simultaneously introducing a gas stream and at least one thread-like inlay into the body in formation, said inlay being pre-treated with a substance capable of so acting upon said body in formation as to obtain an intimate union between the latter and the inlay.
10. A process for making artificial textiles such as hollow threads, tube- or hose-like bodies, artificial straw, flat strips and the like from esters and/or ethers of cellulose, according to the dry method, comprising pressing highly concentrated, dough-like solutions or masses flowing only with difficulty or not at all at ordinary temperature, and containing at least about 30% of cellulose derivative, through nozzles with annular orifices under high pressure, while simultaneously jointly introducing at least one thread-like inlay and a gas stream into the body in formation, and then passing the obtained body through finishing means.
11. A process for making artificial textiles such as hollow threads, tube- or hose-like bodies, artificial straw, flat strips and the like from esters and/or ethers of cellulose, according to the dry method, comprising forcing highly concentrated, dough-like solutions or masses flowing only with difficulty or not at all at ordinary temperature, and containing at least about 30% of cellulose derivative, through nozzles with annular orifices under high pressure, while simultaneously jointly introducing at least one thread-like inlay and a gas stream into the body in formation, and thereupon passing the resultant body over rollers to externally modify its surface.
12. In a process for making artificial textiles such as hollow threads, tube- or hose-like bodies, artificial straw, flat strips and the like from esters and/or ethers of cellulose, according to the dry method, comprising forcing highly concentrated, dough-like solutions or masses flowing only with difficulty or not at all at ordinary temperature, and containing at least about 30% of cellulose derivative, through nozzles with annular orifices under high pressure, while simultaneously jointly introducing at least one textile thread as inlay and a gas stream into the body in formation.
13. In a process for making artificial textiles such as hollow threads, tube- or hose-like bodies, artificial straw, flat strips and the like from esters and/or ethers of cellulose, according to the dry method, comprising forcing highly concentrated, dough-like solutions or masses flowing only with difficulty or not at all at ordinary temperature, and containing at least about 30% of cellulose derivative, through nozzles with annular orifices under high pressure, while simultaneously jointly introducing at least one wire as inlay and a gas stream into the body in formation.
14. In a process for making artificial textiles such as hollow threads, tube- or hose-like bodies, artificial straw, flat strips and the like from esters

and/or ethers of cellulose, according to the dry method, comprising forcing highly concentrated, dough-like solutions or masses flowing only with difficulty or not at all at ordinary temperature, 5 and containing at least about 30% of cellulose derivative and a fine metallic powder as filling substance incorporated in the solutions, through nozzles with annular orifices under high pressure, while simultaneously jointly introducing at 10 least one thread-like inlay and a gas stream into the body in formation.

15. In a process for making artificial textiles such as hollow threads, tube- or hose-like bodies,

artificial straw, flat strips and the like from esters and/or ethers of cellulose, according to the dry method, comprising forcing highly concentrated, dough-like solutions or masses flowing only with difficulty or not at all at ordinary temperature, 80 and containing at least about 30% of cellulose derivative and a coloring matter as filling substance incorporated in the solutions, through nozzles with annular orifices under high pressure, while simultaneously jointly introducing at least 85 one thread-like inlay and a gas stream into the body in formation.

OTTO LAUBI.

90

15

20

95

25

100

30

105

35

110

40

115

45

120

50

125

55

130

60

135

65

140

70

145

75

150